

R. H. HENDERSON.  
PROCESS OF PREPARING METALLIC FILAMENTS.  
APPLICATION FILED DEC. 5, 1910.

1,169,819.

Patented Feb. 1, 1916.



WITNESSES:

C. L. Belcher.  
Otto S. Schaefer.

INVENTOR  
*Robert H. Henderson*  
BY  
*Wiley Clark*  
ATTORNEY

# UNITED STATES PATENT OFFICE.

ROBERT H. HENDERSON, OF EAST ORANGE, NEW JERSEY, ASSIGNOR TO WESTINGHOUSE LAMP COMPANY, A CORPORATION OF PENNSYLVANIA.

## PROCESS OF PREPARING METALLIC FILAMENTS.

1,169,819.

Specification of Letters Patent.

Patented Feb. 1, 1916.

Application filed December 5, 1910. Serial No. 595,629.

To all whom it may concern:

Be it known that I, ROBERT H. HENDERSON, a citizen of the United States, and a resident of East Orange, in the county of Essex and State of New Jersey, have invented a new and useful Improvement in Processes of Preparing Metallic Filaments, of which the following is a specification.

My invention relates to processes of preparing filaments for incandescent lamps and particularly to processes of preparing metallic filaments, such as those composed of, or containing, tungsten.

The object of my invention is to provide a process of treatment by which tungsten and similar metallic filaments may be rendered more tough and durable, and of more compact and homogeneous texture than they are before treatment, or when produced by other processes.

Tungsten is generally recognized as a particularly desirable material for use in the manufacture of filaments for incandescent lamps, because of the very high efficiency of lamps having such filaments, but trouble has been experienced in the use of tungsten, as heretofore produced in the form of filaments, by reason of its brittle and fragile character.

According to the present invention, I propose to subject sintered filamentary tungsten, such as is now ordinarily used for lamp filaments, or another metal or a combination of metals or substances which are not sufficiently ductile at ordinary temperatures for practical purposes, such as titanium, zirconium, uranium, chromium and silicon, to a treatment which will render it much more tough and durable, and generally more satisfactory for use in incandescent lamps than it is before subjection to such treatment. The treatment consists in heating the filamentary material to a high temperature to render it plastic, and at the same time compacting or compressing its particles into a smaller space or diameter, as by drawing it through a die, or swaging it, the filament being thus rendered more compact and homogeneous in texture and its physical character being so modified as to render it more tough.

It has been proposed to reduce tungsten wire to a small diameter by drawing it through dies, while the wire is heated to a low temperature. This, however, is not done

for the purpose of compacting the wire, but is in all respects similar to the ordinary process of drawing fine metal wires through dies, a slight amount of heating being necessary in order to get the tungsten to draw at all, as it is practically non-ductile when cold. It is, therefore, necessary in the said process, as in all wire-drawing operations, to employ a great number of dies in order to reduce the cross-section of the material very gradually. The present invention, however, differs essentially in principle from the process described above, the purpose being to force the individual metallic particles composing the filament into very close contact, or in other words, to obtain a close actual welding together of these particles, which can only be gotten by subjecting them to a mechanical compacting process, such as drawing through a die, at a high temperature, while the particles are in a highly plastic condition, so that they can easily weld together. On this account the aim is not to obtain a very gradual, but rather a sudden reduction of the original diameter of the filament under treatment, and this can be attained on account of the high temperature at which the operation is carried out.

The single figure of the accompanying drawing is a view, in elevation and in section, of simple and suitable apparatus for practising my invention.

The filamentary material 1, to which the treatment of the present invention is applied, may be obtained from any suitable source, in either short or long lengths, as desired, but I prefer to use filamentary material that is produced continuously and in great lengths by the process and machine set forth in an application Serial No. 486,925, filed March 31, 1909, by Harry D. Madden, and William G. Houskeeper, assigned to the Westinghouse Lamp Company, and patented June 2, 1914, No. 1,099,095, and I also prefer to attach the means for practising my process directly to the machine set forth in the said patent. The purer the material that is used in the operation of this machine, the better will be the results obtained by its use, particularly in connection with the present process. The filamentary material obtained from the said machine or otherwise may be passed through two spaced and apertured terminal devices 2 and 3 that

are suitably connected to an electric circuit 4—5, and the apertures of which are filled with mercury that is held in place by its surface tension and its capillary attraction 5 for the edges of the aperture, which are preferably amalgamated. A current passed through the filament from the one terminal device to the other raises the temperature of the intermediate portion of the filament to 10 the required degree. While the filamentary material is thus heated it is passed through one or more dies 6 having apertures of smaller diameter than that of the filamentary material in its original condition. In 15 order to start the filamentary material through the die, its end **must** be reduced in diameter to something less than that of the aperture in the die, and, to this end, it may be heated and stretched or compressed, or 20 it may be treated chemically, as by partial oxidation, in order to remove its outer portions. The filament may be drawn through the die by applying tension to it at its lower end by any suitable means, such as a weight 25 upon which gravity acts, or by means of any suitable mechanical device.

The compacting of the filament, while highly heated, may be effected by other means than a die, if desired, as by swaging, 30 by impact, or otherwise, and the filamentary material may be heated otherwise than electrically.

The physical characteristics of the filamentary material may be improved not only 35 by its mechanical compacting at a high temperature either before or after the application to it of a sintering temperature, but also

by the application to it after it is sintered of a thermal treatment adapted to effect the desired physical changes, such as 40 rendering it more ductile and pliable.

I claim as my invention:

1. The process of preparing filamentary structures containing a metal having a high fusing point which consists in first 45 producing the material in filamentary form, and then heating the same while mechanically working it.

2. The process of preparing filamentary structures consisting of a metal having a 50 high fusing point which consists in first producing the material in filamentary form and then heating the same to a high temperature and mechanically compacting it while heated.

3. The process of treating filamentary structures containing a metal having a high fusing point which consists in heating the same to a high temperature and mechanically compacting it while heated.

4. The process of treating filamentary structures containing a metal having a high fusing point which consists in passing an electric current through it to heat it to a high temperature and mechanically compacting it while heated.

In testimony whereof, I have hereunto subscribed my name this 23rd day of November, 1910.

ROBERT H. HENDERSON.

Witnesses:

OTTO S. SCHAIRER,  
CHARLES E. KELLY.